

No. 778,136.

PATENTED DEC. 20, 1904.

P. MAGNUS.

PNEUMATIC TIRE.

APPLICATION FILED OCT. 5, 1904.

NO MODEL.



Fig. 1.



Fig. 2.



Fig. 3.



Fig. 4.



Fig. 5.



Fig. 6.

Witnesses:  
James D. Mansfield.  
L. E. Watham.

Inventor:  
Philip Magnus.  
By: Alexander T. Powell  
Attorneys.

## UNITED STATES PATENT OFFICE.

PHILIP MAGNUS, OF NORTHCOTE, VICTORIA, AUSTRALIA.

## PNEUMATIC TIRE.

SPECIFICATION forming part of Letters Patent No. 778,136, dated December 20, 1904.

Application filed October 5, 1904. Serial No. 227,227.

*To all whom it may concern:*

Be it known that I, PHILIP MAGNUS, a subject of the King of Great Britain and Ireland, residing at 27 Harper street, in the town of Northcote, in the county of Bourke, State of Victoria, and Commonwealth of Australia, have invented certain new and useful Improvements in Pneumatic Tires, of which the following is a specification.

10 The object of my invention is to provide a pneumatic-tire cover which shall not only be cheap, but also strong, durable, and resilient.

The ordinary leather covers are inert and lack resiliency, which militates greatly against them, while the liability of india-rubber covers to puncture is a serious objection; but with my present invention, which is an improvement on my prior patent, No. 740,578, the advantages of leather and rubber are combined without the disadvantages to which they are subject when separated.

Referring to the drawings which form a part of this specification, Figure 1 represents a section of a cycle-tire with my invention applied. Fig. 2 shows in section my invention as applied to a motor-cycle tire. Fig. 3 represents a tire-cover built according to my invention and suitable for light or medium motor-cars. Fig. 4 depicts a cover suitable for heavy cars. Fig. 5 represents in section a side elevation of one of my solution-impregnated circumferential segments. Fig. 6 shows a section of Fig. 5. Fig. 7 depicts a side elevation of a number of my solution-impregnated circumferential segments placed end to end.

Similar letters of reference indicate similar or corresponding parts where they occur in the several views.

40 My invention includes a hide which is "split" into two sheets of leather—the "skin," or outer, and the "flesh," or inner, portion. I do not use the skin portion; but the cheaper flesh portion is then treated in any well-known way to remove therefrom excess of grease or other impurities. The cleansed leather is then cut into the strips or circumferential segments marked A in the drawings. These in length are as long as possible, and their width will

50 depend upon the diameter of the tire and

other conditions. These strips are then immersed for twelve hours (more or less) in a solution of mineral naphtha and caoutchouc or india-rubber. This solution consists approximately of seventy (70) per cent. of naphtha and thirty (30) per cent. of rubber. While immersed they are subjected to moderate movement and, if necessary, may be placed on edge. Each strip is then introduced to a pricking and impregnating machine. This consists of two rollers, one above the other or side by side. These rollers (the distance between which is adjustable) are one-eighth ( $\frac{1}{8}$ ) of an inch apart, (more or less,) and the circumference of one or of both is studded with 60 prickers. The area, length, and section of these will depend upon circumstances. For some leathers they may be round and pointed, while for others they may be square or of other section and unpointed. With some 70 leathers the prickers are neither pointed nor parallel, but larger at the point than at the root. Upon these rollers falls or is sprayed a solution of approximately sixty (60) per cent. of naphtha and forty (40) per cent. of rubber. 75 The rollers are therefore covered with solution, and as the prickers leave the leather the solution enters. A collector below gathers the overflow solution for reuse.

Instead of the circumferential segments 80 passing between rollers they may be placed beneath a stamp from below which prickers protrude. The said prickers are hollow and perforated, and through the perforations the solution is forced into the leather before the 85 prickers are withdrawn.

After pricking, the strips are immersed for twelve hours (more or less) in a solution of approximately sixty (60) per cent. of naphtha and forty (40) per cent. of rubber. After the 90 foregoing immersion each strip is reduced at each end, as seen in Fig. 5, to represent a wedge. At the left-hand end is the upper wedge-point B, and at the right-hand end is the lower wedge-point C. Each strip has also its side edges 95 reduced, as seen at the side-edge reductions D. Said strips are then allowed to partially dry. An endless fabric or band E is then laid upon the circumference of a circular mold or former. The outer surface of the fabric is cov- 100

ered with an adhesive and the edges F folded back upon the said outer surface, inclosing a wire or ring G or a clenching-ring H. The fabric is then removed from the former and 5 its outer surface treated at suitable intervals with further solutions of naphtha and rubber. The fabric is then replaced on the former, and an inner composition J, approximately twenty (20) per cent. of naphtha and eighty (80) per 10 cent. of rubber, is applied to its circumference. The thickness and width of this will depend upon the purposes for which the tire is to be used. One by one the circumferential segments A are then applied to the composition, an upper wedge-point B being placed 15 over a lower one C. A circle is thus completed formed by a series of segments. Between eachlapping joint thus formed an adhesive solution is applied. On the exterior 20 of the circumferential segments another layer K of the last composition is applied, the thickness and width of which will depend upon conditions. This is hereinafter called the "outer" 25 composition K. The cover thus formed is ready for the application thereto of heat and pressure, whereby all the parts are completely united. When completed, the cover is attached to the rim M and covers the air-tube 30 N. For heavier tires another ring, an outer 35 ring A' of circumferential segments, is applied to the composition K. Outside this is placed another ring, L, of composition, hereinafter called the "outermost" composition. I do not bind myself to the number of the said rings of circumferential segments.

For heavier tires the reduced edges of the circumferential segments instead of only covering the tread, as seen in Fig. 1, extend to and below the walls of the tire, as seen in Figs.

40 2 and 4.

Having now described my invention, what I claim as new, and desire to secure by Letters Patent, is—

1. In pneumatic tires a series of segments 45 formed of "flesh" leather, said segments having been immersed in a solution approximately of seventy (70) per cent. of naphtha and thirty (30) per cent. india-rubber, then passed between rollers having prickers and a solution 50 of approximately sixty (60) per cent. naphtha and forty (40) per cent. india-rubber on the rollers, then immersed in a solution approximately of sixty (60) per cent. naphtha and forty (40) per cent. india-rubber, each segment having 55 its sides reduced and its edges wedge-pointed all as and for the purpose hereinbefore described.

2. A pneumatic-tire cover comprising an inner layer or fabric, a circumferential series 60 of leather segments surrounding said inner layer each segment having been impregnated with a solution of approximately sixty per cent. of mineral naphtha and forty per cent. of

rubber; and an outer layer formed of a composition of approximately twenty per cent. of 65 mineral naphtha and eighty per cent. of rubber, the aforesaid parts being subjected to heat and pressure to unite them, substantially as and for the purposes described.

3. A cover for pneumatic tires formed of 70 an inner layer of fabric, a composition around said layer formed of approximately twenty percent. of mineral naphtha and forty percent. of rubber; a series of leather segments encircling said fabric, each segment having been 75 impregnated with a solution of approximately sixty percent. of mineral naphtha and forty percent. of rubber; and an outer composition of approximately twenty per cent. of mineral naphtha and eighty per cent. of rubber; said 80 fabric, composition, segments and outer composition being united by heat and pressure, substantially as and for the purpose described.

4. In pneumatic tires a cover formed of an endless fabric, a composition around said fabric approximately of twenty (20) per cent. mineral naphtha and forty (40) per cent. rubber, outside said fabric a series of "flesh" leather circumferential segments forming a circle, each segment having reduced side 90 edges, an upper wedge-point at one end, a lower wedge-point at the other, said segment having been pricked and impregnated with a solution of approximately sixty (60) per cent. of mineral naphtha and forty (40) per cent. of rubber, an outer composition of approximately twenty (20) per cent. of mineral naphtha and eighty (80) per cent. of rubber, around 95 said segments, said fabric, composition, segments and outer composition being subjected to heat and pressure, all as and for the purposes hereinbefore described.

5. In pneumatic tires a cover formed of an endless fabric, a wire, or clenching-ring inclosed in each edge, an inner composition of 105 approximately twenty (20) per cent. mineral naphtha and eighty (80) per cent. rubber around the fabric, inner circumferential "flesh" leather segments having their side edges reduced and at one end an upper wedge-point and at the other a lower wedge-point, said wedge-points being united by an adhesive, said segments having been pricked and impregnated and forming a ring, an outer composition of approximately twenty (20) per cent. mineral naphtha and eighty (80) per cent. rubber, an outer ring of segments, and an outermost composition, all as and for the purposes hereinbefore described.

In witness whereof I have hereunto set my hand to this specification in the presence of two witnesses.

PHILIP MAGNUS.

Witnesses:

EDWIN PHILLIPS,  
CECIL W. LE PLASTRIER.